

# United States Patent [19]

Terada et al.

[11]

4,353,979

[45]

Oct. 12, 1982

[54] **LIGHT-SENSITIVE SILVER HALIDE PHOTOGRAPHIC MATERIALS**

[75] Inventors: **Sadatugu Terada; Hideaki Arai, both of Hachioji; Kenji Itoh, Hino; Hiroshi Sugita, Hachioji; Katsumi Matsuura, Akigawa; Thuneo Wada, Sagamihara, all of Japan**

[73] Assignee: **Konishiroku Photo Industry Co., Ltd., Tokyo, Japan**

[21] Appl. No.: **169,423**

[22] Filed: **Jul. 16, 1980**

[30] **Foreign Application Priority Data**

Jul. 25, 1979 [JP] Japan ..... 54-95233

[51] Int. Cl.<sup>3</sup> ..... **G03C 7/00; G03C 1/40**

[52] U.S. Cl. ..... **430/372; 430/377; 430/382; 430/449; 430/512; 430/544; 430/546; 430/548; 430/554; 430/957**

[58] **Field of Search** ..... 430/377, 493, 382, 372, 430/512, 546, 601, 610, 449, 544, 548, 554, 957

[56] **References Cited**

U.S. PATENT DOCUMENTS

2,322,027 12/1940 Jolley et al.

|           |         |                      |
|-----------|---------|----------------------|
| 3,258,338 | 6/1966  | Claeys et al.        |
| 3,544,336 | 12/1970 | Milton .....         |
| 3,554,755 | 1/1971  | Rinauro .....        |
| 3,676,137 | 7/1972  | Mizuki et al. ....   |
| 4,220,711 | 9/1980  | Nakamura et al. .... |

430/610  
430/377  
430/546

**FOREIGN PATENT DOCUMENTS**

48-32727 8/1973 Japan .....

*Primary Examiner*—J. Travis Brown  
*Attorney, Agent, or Firm*—Finnegan, Henderson, Farabow, Garrett & Dunner

[57]

**ABSTRACT**

A silver halide photographic material containing a solution of a 5-pyrazolone type magenta coupler and a high-boiling organic solvent of the formula:



wherein R<sub>1</sub>, R<sub>2</sub> and R<sub>3</sub> each represent an aliphatic or aromatic group with a carbon atom of R<sub>3</sub> directly bonded to the phosphorus atom.

**8 Claims, No Drawings**

## LIGHT-SENSITIVE SILVER HALIDE PHOTOGRAPHIC MATERIALS

This invention relates to light-sensitive silver halide photographic materials in general and more particularly to light-sensitive silver halide color photographic materials, wherein hydrophilic colloidal solutions for forming constitutive layers of said photographic materials are individually incorporated with a variety of oil-soluble photographic additives, such as photographic couplers or the like, each being dissolved and dispersed in high boiling organic solvents.

In the course of preparing light-sensitive silver halide photographic materials of every kind, various photographic additives are incorporated into hydrophilic colloidal solutions for forming constitutive layers of said photographic materials. In a process of incorporating such photographic additive into hydrophilic colloidal solution, generally the additive previously dissolved in water or a solvent therefor, such as an organic solvent, is added to said solution. In point of its ability as a solvent without ill effect on photographic characteristics, etc. of the resulting light-sensitive silver halide photographic material, water is the best for dissolving photographic additives for the incorporation thereof into said photographic material. Generally, however, numerous photographic additives are difficultly soluble in water, and for dissolving such additives there are used lower alcohols, such as methanol, ethanol, etc., acetone or mixtures thereof with water. However, there are a good many of photographic additives which are also difficultly soluble even in such organic solvents as mentioned above. Typical of these so-called oil-soluble photographic additives are, for example, couplers, DIR compounds, ultraviolet absorbers, photofading inhibitors, color staining inhibitors, etc. As one of processes for incorporating such oil-soluble photographic additives into layers constituting light-sensitive silver halide photographic materials, such as silver halide emulsion layers, auxiliary layers and the like, it is known to incorporate into coating solutions for such constitutive layers the additives in the form of a dispersion comprising fine droplets consisting of an organic solvent immiscible with water, in which fine droplets said additives have individually been dissolved as solute. Such organic solvents as may be used for the above purpose are desired to meet the following requirements. That is, the organic solvent is such that it is miscible with oil-soluble photographic additives, preferably it is substantially capable of dissolving the oil-soluble photographic additives and also capable of permeating into developing solutions, that it does not bring about crystallization of the oil-soluble photographic additive contained therein to cause precipitation or aggregation thereof and is capable of keeping the aforesaid small droplets stably dispersed, that it has a refractive index which is as close as possible to that of a hydrophilic binder in which it has been dispersed, and that it does not soften or weaken layers in which it is to be contained by dispersion and also does not deteriorate the layers in physical properties.

As organic solvents used for dispersing and containing oil-soluble photographic additives in the form of fine droplets thereof in constitutive photographic layers, there have heretofore been known a variety of high boiling organic solvents as disclosed in U.S. Pat. Nos. 2,322,027 and 3,554,755. By way of example, there may

be mentioned, for example, phthalates of methyl, ethyl, butyl, benzyl, nonyl and decyl, benzoates of benzyl, butyl-o-methoxy and n-hexyl, triphenyl phosphate, tricresyl phosphate, p-toluenesulfonyldimethylamide, benzophenone, acetophenone, tetrahydrofurfuryl succinate, ethyl succinate, ethanolamine and the like.

However, all oil-soluble photographic additives are not always excellently soluble in the above-mentioned high boiling organic solvents. For instance, couplers or some additives are poor in dispersion stability when they are dispersed by the use of such high boiling organic solvents, and they tend to crystallize or bring about aggregation thereof at any stage of process steps, for example, when they are subjected to emulsification and dispersion by means of a colloid mill or homoblender, while they are on standing after having been incorporated into emulsions or gelatin solutions, and at the time of their being coated and dried, thereby causing sometimes uneven coating and deterioration in image quality. Furthermore, high boiling organic solvents capable of sufficiently dissolving couplers, ultraviolet absorbers or the like additives are generally not always favorable in dispersion stability. Of the conventionally used high boiling organic solvents, some are found poor in dispersion stability even though they have high dissolving power, and on that account such solvents often bring about crystallization aggregation thereof at any stage of the process steps as aforesaid.

In recent years, the conventionally used high boiling organic solvent often throw a hindrance from coloration of couplers in some cases where a strict condition control of the developing treatment of exposed photographic materials at high temperatures with rapidity as well as of the treatment free from environmental pollution is increasingly required.

The use of alkyl phosphate ester high boiling solvents as disclosed in Japanese Patent Publication No. 32727/1973 is known for the purpose of obviating the above-mentioned drawbacks associated with the prior art, wherein a further improvement in color purity is intended by the reduction of subabsorption in red light region resulting from shifting the principal absorption wavelength of magenta forming dyes to a shorter wavelength. In the use of these alkyl phosphate ester solvents as the high boiling solvents for aldehydebis type 5-pyrazolone magenta couplers, however, there is certainly observed an improved high ability to dissolve the couplers or the alleged effect obtained by shifting the principal wavelength of the magenta forming dyes to the shorter one. On the other hand, there are brought about such drawbacks that stability of the couplers during development treatment is not satisfactory and unexposed photographic films having contained therein the couplers are found poor in storage stability, and a hindrance for coloration by the coupler is brought about.

Accordingly, a first object of the present invention is to provide light-sensitive silver halide photographic materials wherein the oil-soluble photographic additives intended to be used can stably be contained in hydrophilic colloid liquid without coagulation used for constituting layers on said photographic materials while dispersing said photographic additives in said colloid solution.

A second object of the present invention is to provide light-sensitive silver halide color photographic materials wherein color developability of the couplers used has been improved without formation of fog.

A third object of the present invention is to provide light-sensitive silver halide color photographic materials wherein the color images formed thereon have been improved in stability during storage (fastness to light, heat and humidity).

A fourth object of the present invention is to provide light-sensitive silver halide color photographic materials wherein the colored dyes formed by means of 5-pyrazolone magenta couplers have been improved in spectral absorption property.

A fifth object of the present invention is to provide light-sensitive silver halide color photographic materials wherein stability during development treatment of aldehydebis type 5-pyrazolone magenta couplers has been improved.

A sixth object of the present invention is to provide light-sensitive silver halide color photographic materials containing aldehydebis type 5-pyrazolone magenta couplers with an improved stability.

In the present invention the oil-soluble photographic additives are dissolved by the use of a compound represented by the following general formula, then the obtained solution is dispersed into hydrophilic colloid liquid which is incorporated in constituting layers of light-sensitive silver halide photographic materials.

General formula [I]



In the formula  $\text{R}_1$ ,  $\text{R}_2$  and  $\text{R}_3$  each represent an aliphatic or aromatic group (e.g. carbocyclic rings, heterocyclic rings, etc.), and  $\text{R}_3$  shows that the carbon atom thereof is bonded directly to the phosphorus atom. Preferably,  $\text{R}_1$ ,  $\text{R}_2$  and  $\text{R}_3$  each represent an alkyl or aryl group and  $\text{R}_1$ ,  $\text{R}_2$  and  $\text{R}_3$  may be the same or different if the sum total of carbon atoms of  $\text{R}_1$ ,  $\text{R}_2$  and  $\text{R}_3$  is in the range from 6 to 50. More preferably,  $\text{R}_1$  and  $\text{R}_2$  is each 40 an alkyl, acyl, alkoxyalkyl, aryloxyalkyl or aryl group of 1 to 20 carbon atoms, each of these substituents may be further substituted by other substituent.  $\text{R}_3$  may be a carbonyloxy- or carbonamido-containing group (e.g. alkoxy carbonylalkyl, acyloxyalkyl, acyloxyaryl, alkylaminocarbonylalkyl, acylaminoalkyl or the like group), alkoxyalkyl, aryloxyalkyl, alkoxyaryl, arylalkyl or acylalkyl.

That is, by virtue of the use of at least one of the compounds represented by the above-mentioned general formula [I], satisfactory dispersion stability can be attained in couplers, ultraviolet absorbers and other oil-soluble photographic additives used in light-sensitive silver halide photographic materials without bringing about unevenness in coating or deterioration in image quality. When the compounds of the general formula [I] are used in the preparation of light-sensitive silver halide color photographic materials, moreover, excellent fastness to light, heat and/or humidity can be imparted to the dye images resulting from color development treatment of said photographic materials.

Some of the conventional couplers and other oil-soluble photographic additives were known to exhibit excellent performances in various points. Nevertheless, they were in most cases difficult to put them to practical use because of being difficultly soluble in and having poor dispersion stability in every high boiling organic solvents hitherto known. However, by virtue of the use

of the high boiling organic solvents according to the present invention, such known couplers or oil-soluble photographic additives as having excellent properties as aforesaid have, in fact, come to be satisfactorily used without the least inconvenience, and thus this is a great significance in practical sense of the present invention.

Further, many of the conventionally used high boiling organic solvents are liable to an increased fog formation in the resulting silver halide emulsions or to formation of stain or discoloration in white ground of the uncolored area of the resulting light-sensitive silver halide color photographic after color development. The high boiling organic solvents used in the present invention, however, are in no way suffering from such inconveniences.

Of late years, it has been commonly practiced to make thinner photosensitive layers of light-sensitive silver halide photographic materials in order to improve the photographic materials in their characteristics so as to be able to meet high temperature and quick photographic processing techniques to which said materials are inevitably applied. As one of the means of making the photosensitive layers thinner, there is a procedure of reducing the quantity of a high boiling organic solvent to be used in said photosensitive layers. As the result, there were observed many cases where a hindrance to development of color by means of the couplers was brought about owing to the reduction of quantity of the conventionally used high boiling organic solvents for that purpose. In the case of the high boiling organic solvents used in the present invention, however, no such inconvenience is anticipated at all.

Concrete examples of the high boiling organic solvents represented the aforesaid general formula and used in the present invention are exemplified below.

| Compound No. | Formula                                                                                                                    |
|--------------|----------------------------------------------------------------------------------------------------------------------------|
| 1            | $\text{C}_{12}\text{H}_{25}\text{P}(\text{O})(\text{OC}_2\text{H}_5)_2$                                                    |
| 2            | $\text{C}_{12}\text{H}_{25}\text{OCH}_2\text{CH}_2\text{CH}_2\text{P}(\text{O})(\text{OC}_2\text{H}_5)_2$                  |
| 3            | $\text{CH}_3\text{COOCH}_2\text{CH}_2\text{P}(\text{O})(\text{OC}_2\text{H}_5)_2$                                          |
| 4            | $(\text{BuO})_2\text{P}(\text{O})(\text{CH}_2\text{COOC}_2\text{H}_5)_2$                                                   |
| 5            | $\text{EtOCH}_2\text{P}(\text{O})(\text{OC}_3\text{H}_7)_2$                                                                |
| 6            | $\text{CH}_3\text{COCH}_2\text{C}(\text{CH}_3)_2\text{P}(\text{O})(\text{OC}_3\text{H}_7(\text{iso}))_2$                   |
| 7            | $\text{CH}_3\text{OCH}_2\text{CH}_2\text{COCH}_2\text{C}(\text{CH}_3)_2\text{P}(\text{O})(\text{OC}_2\text{H}_5)_2$        |
| 8            | $\text{CH}_3\text{O}(\text{CH}_2)_3\text{COCH}(\text{CH}_3)\text{CH}_2\text{P}(\text{O})(\text{OCH}_3)_2$                  |
| 9            | $\text{C}_6\text{H}_{13}\text{P}(\text{O})(\text{OC}_2\text{H}_5)_2$                                                       |
| 10           | $\text{C}_8\text{H}_{17}\text{P}(\text{O})(\text{OC}_4\text{H}_9)_2$                                                       |
| 11           | $\text{C}_{10}\text{H}_{21}\text{P}(\text{O})(\text{OC}_4\text{H}_9)_2$                                                    |
| 12           | $\text{C}_{14}\text{H}_{29}\text{P}(\text{O})(\text{OCH}_3)_2$                                                             |
| 13           | $\text{C}_4\text{H}_9\text{P}(\text{O})(\text{OC}_4\text{H}_9)_2$                                                          |
| 14           | $\text{C}_5\text{H}_{11}\text{P}(\text{O})(\text{OC}_4\text{H}_9)_2$                                                       |
| 15           | $\text{iso-C}_8\text{H}_{17}\text{P}(\text{O})(\text{OC}_4\text{H}_9)_2$                                                   |
| 16           | $\text{CH}_3\text{P}(\text{O})(\text{O}-\text{C}_6\text{H}_4-\text{O})_2$                                                  |
| 17           | $\text{CH}_3\text{P}(\text{O})(\text{OC}_3\text{H}_7)_2$                                                                   |
| 18           | $\text{C}_6\text{H}_5\text{CH}_2\text{CH}=\text{CHCH}_2\text{P}(\text{O})(\text{OC}_2\text{H}_5)_2$                        |
| 19           | $\text{Cl}-\text{C}_6\text{H}_4-\text{CH}_2\text{C}(\text{CH}_3)=\text{CHCH}_2\text{P}(\text{O})(\text{OC}_2\text{H}_5)_2$ |
| 20           | $\text{CH}_3\text{P}(\text{O})(\text{OC}_3\text{H}_7)(\text{OC}_6\text{H}_{13})$                                           |
| 21           | $\text{C}_6\text{H}_5\text{P}(\text{O})(\text{OCH}_3)_2$                                                                   |

-continued

| Compound No. | Formula                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                      |
|--------------|--------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------|
| 22           |                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                             |
| 23           |                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                             |
| 24           |                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                             |
| 25           | $C_8H_{17}P(O)(OC_8H_{17})_2$                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                |
| 26           | $C_2H_5OCO(CH_2)_{10}P(O)(OC_2H_5)_2$                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                        |
| 27           | $C_{12}H_{25}OCO(CH_2)_{10}P(O)(OC_{12}H_{25})_2$                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                            |
| 28           | $C_4H_9CH(C_2H_5)CH_2OCO(CH_2)_{10}P(O)(OC_4H_9)_2$                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                          |
| 29           | $CH_3(CH_2)_7CH(CH_2)_8COOC_2H_5$<br>P(O)(OC2H5)2                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                            |
| 30           | $CH_3(CH_2)_7CH(CH_2)_8COOCH_2CH(C_2H_5)C_4H_9$<br>P(O)(OCH2CH(C2H5)C4H9)2                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                   |
| 31           | $CH_3(CH_2)_7COOCH_2CH_2P(O)(OC_2H_5)_2$                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                     |
| 32           | $CH_3(CH_2)_{12}COOCH_2CH_2P(O)(OC_4H_9)_2$                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                  |
| 33           | $CH_3(CH_2)_5CH-COOC_2H_5$<br>P(O)(O-  -CH3)2                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                               |
| 34           | $CH_3(CH_2)_9CHCOOCH_2CH(C_2H_5)C_4H_9$<br>P(O)(OC2H5)2                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                      |
| 35           | $CH_3(CH_2)_5CHCOOC_4H_9$<br>P(O)(OC6H13)2                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                   |
| 36           | $CH_3(CH_2)_{11}CHCON(C_2H_5)_2$<br>P(O)(OC2H5)2                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                             |
| 37           | $CH_3(CH_2)_5CHCOO-\img alt="Benzene ring" data-bbox="535 595 595 625"/>$<br>P(O)(OC2H5)2                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                    |
| 38           |                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                           |
| 39           | $(C_2H_5O)_2P=CHCOOCH_2CHC_4H_9$<br>  <br>$OCH_2COOCH_2CHC_4H_9$<br>  <br>$C_2H_5$                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                           |
| 40           | $(C_4H_9O)_2P=CH_2-CHCOOC_4H_9$<br>  <br>$O$<br>$CH_2COOC_4H_9$                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                              |
| 41           |  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  -O-  - |

-continued

| Compound<br>No. | Formula                                                                                                                                              |
|-----------------|------------------------------------------------------------------------------------------------------------------------------------------------------|
| 5<br>43         | $\text{H}_9\text{C}_4-\overset{\text{O}}{\underset{  }{\text{P}}}-\text{O}-\text{C}_6\text{H}_4-\text{CH}_3)_2$                                      |
| 10<br>44        | $\text{H}_9\text{C}_4\text{O}(\text{CH}_2)_2-\overset{\text{O}}{\underset{  }{\text{P}}}-\text{O}-\text{C}_6\text{H}_4)_2$                           |
| 15<br>45        | $\text{H}_{17}\text{C}_8\text{O}(\text{CH}_2)_2-\overset{\text{O}}{\underset{  }{\text{P}}}-\text{O}-\text{C}_6\text{H}_4-\text{C}_4\text{H}_9(t)_2$ |
| 20<br>46        | $\text{H}_9\text{C}_4\text{OCO}(\text{CH}_2)_4-\overset{\text{O}}{\underset{  }{\text{P}}}-\text{O}-\text{C}_6\text{H}_4-\text{CH}_3)_2$             |

These high boiling solvents of the present invention as exemplified above may be synthesized according to the procedures as disclosed in the following literatures.

25 respectively: BP. 694,772 J Am Chem Soc 79 6524 (1957) J Am Chem Soc 81 6275, J Org Chem 25 1000 (1960), Radiochim Acta 8 (2), 102-6 (1967), Zh Obshch Khim 1968 38 (5) 1112-16, Zh Obshch Khim 1968 38 (6) 1278-82, Zh Obshch Khim 22 920-6 (1952), Zh Obshch Khim 22 1143-7 (1952), Zh Obshch Khim (J Geu Chem) 22 914-20 (1952) J Am Chem Soc 79 3570 (1957), Org Synth 31 33 (1951), J Am Chem Soc 75 3379 (1953), J Am Chem Soc 1953 2224, J Chem Soc 1964 4369, J Am Chem Soc 67 1180 (1945) and U.S. Patent No. 3,258,338.

Illustrated below are synthesis examples of some of the above-exemplified compounds which are preferably usable in the present invention.

## Synthesis Examples

### Compound 1

A mixture comprising 24.7 g of 1-octene, 61.8 g of diethyl phosphite and 0.3 g of benzoyl peroxide was allowed to undergo reaction at 80°–85° C. for 15 hours.

45 In the course of the reaction, 0.3 g of benzoyl peroxide was further added to the system. After the completion of the reaction, the reaction liquid was distilled under reduced pressure to obtain 34.1 g of diethyl-1-octane phosphonate, b.p.  $105^{\circ}\text{--}106^{\circ}\text{ C.}$  /0.8 mm Hg.

### Compound 5

A mixture comprising 45 g of tributyl phosphite and 25 g of bromomethyl ethyl ether was allowed to undergo reaction at 150°-160° C. for 1.5 hours. After the completion of the reaction, the reaction liquid was distilled under reduced pressure to obtain 30.0 g of butylethoxymethyl phosphonate, b.p. 143°-143.5° C./19 mm Hg.

### Compound 33

A mixture comprising 17.6 g of ethyl  $\alpha$ -bromo-n-caprylate and 23.3 g of triethyl phosphite was allowed to undergo reaction at 160°-190° C. for 7 hours. After the completion of the reaction, the reaction liquid was distilled under reduced pressure to remove excess triethyl phosphite, and the residue was distilled under reduced pressure to obtain 14.5 g of  $\alpha$ -phosphonic acid ester, b.p. 132° C./0.3 mm Hg.

For making dispersions of oil-soluble photographic additives by the use of high boiling organic solvents used in the present invention, the following procedure may be taken with satisfactory results. That is, the oil-soluble photographic additive to be dispersed is first dissolved in the high boiling organic solvent according to the present invention to obtain a solution. This solution is then emulsified by means of a colloid mill, homoblender or the like in an aqueous solution of a hydrophilic protective colloid such as gelatin in the presence of a surface active agent, for example, anionic surfactants such as alkylbenzenesulfonic acids, nonionic surfactants, such as saponin or cationic surfactants such as quaternary ammonium salts of alkylamines. Thereafter, the emulsified dispersion thus obtained may be incorporated into gelatino-silver halide emulsions or aqueous solutions of a hydrophilic protective colloid for use for forming auxiliary layers (intermediate, antihalation, protective and the like layers), followed by uniform dispersing. As an alternative thereto, under certain circumstances, the solution of the oil-soluble photographic additive in the high boiling organic solvent may be incorporated directly into coating solutions for use in forming constitutive layers of light-sensitive silver halide photographic materials, followed by emulsifying and dispersing. In the present invention, however, for the purpose of dispersing oil-soluble photographic additives the high boiling organic solvent according to the present invention represented by the aforesaid general formula [I] in combination with other known high boiling solvents, though such dispersing purposes can sufficiently be attained by the use of the present high boiling organic solvent alone. If necessary, the present high boiling organic solvent can be used in combination with low boiling organic solvents used as co-solvents. Usable as low boiling organic solvents in combination with the present high boiling organic solvents, are those as disclosed, for example in U.S. Pat. Nos. 2,801,170, 2,801,171 and 2,949,360. By way of example, such low boiling organic solvents include methyl isobutyl ketone,  $\beta$ -ethoxyethyl acetate, methoxytriglycol acetate, acetone, methyl acetone, methanol, ethanol, acetonitrile, dioxane, dimethylformamide, dimethyl sulfoxide, ethyl acetate, butyl acetate, isopropyl acetate, butanol, chloroform, cyclohexane, cyclohexanol, fluorinated alcohol, etc.

The high boiling organic solvents used for the present invention may be used in any amounts suitably selected according to the couplers, ultraviolet absorbers or other oil-soluble photographic additives. In such case, however, the use of the present high boiling organic solvents in excessively large amounts is undesirable. For instance, in integral multi-layered light-sensitive silver halide photographic materials, when the present solvents are made present in large amounts in an emulsion layer provided at the upper position of said photographic materials and/or ultraviolet absorber containing layer, developability of an emulsion layer provided at the lower position of said photographic materials is lowered and, furthermore, emulsion layers and gelatin layers containing the solvents in large excess sometimes are deteriorated in their physical properties. Thus, it is appropriate to use the high boiling organic solvent in such a manner that the weight ratio of the present sol-

vent to each oil-soluble photographic additive is substantially in the range of 0.1 to 8.0.

Hydrophilic colloidal liquid for forming constitutive layers of photographic materials, said colloidal liquid having contained therein oil-soluble photographic additives according to the present invention, are coated on a suitable support, for example, plastic films, resin-coated papers, baryta papers, etc, and then dried.

Gelatino-silver halide emulsions are usually most typical of the silver halide emulsions which are used for the performance of the present invention. In the present invention, however, there may also be used such silver halide emulsions having used therein acetylated gelatin, phthalated gelatin, water-soluble cellulose derivatives, other hydrophilic synthetic or natural high molecular compounds, or mixtures thereof with gelatin. Even in the case where the aforesaid hydrophilic colloid liquids for forming the constitutive layers photographic materials are used as hydrophilic protective colloid for forming auxiliary layers other than the silver halide emulsions, other protective colloid as aforesaid may be used therein, though gelatin is used commonly.

Couplers usable in the present invention include all of those which are conventionally known as photographic couplers. Preferably usable couplers include, for example,  $\alpha$ -benzoylacetanilide type yellow couplers,  $\alpha$ -pivaloylacetanilide type yellow couplers, 5-pyrazolone type magenta couplers, pyrazolinobenzimidazole type magenta couplers, phenol type cyan couplers and naphthol type cyan couplers.

The alpha-acylacetamide yellow forming couplers used in the present invention may be synthesized according to procedures respectively disclosed, for example, in West German Laid-Open Patents Nos. 2,057,941 and 2,163,812, Japanese Laid-Open-to-Public Publications Nos. 26133/1972 and 29432/1973, U.S. Pat. Nos. 3,227,550, 2,875,057 and 3,265,506, and Japanese Laid-Open-to-Public Publications Nos. 66834/1973, 66835/1973, 94432/1973, 1229/1974, 10736/1974, 34232/1975, 65231/1975, 117423/1975, 3631/1971 and 50734/1976.

The alpha-acyacetamide yellow forming couplers may be incorporated, either singly or in mixture of two or more, into silver halide emulsion layers, and the incorporation of the coupler in an amount of 5 to 30 mol% per mole of blue-sensitive silver halide can be carried out according to the usual method.

Cyan forming couplers usable in the present invention may be synthesized according to procedures as disclosed, for example, in British Patent Specification No. 1,084,480, Japanese Laid-Open-to-Public Publications Nos. 117422/1975, 10135/1975, 37647/1976, 25228/1975 and 130441/1975. Two equivalent cyan forming couplers are incorporated into silver halide emulsions, either singly or in mixture of two or more, or in admixture with so-called colored couplers, of which the active points have been arylazo-substituted, as disclosed in U.S. Pat. No. 3,034,892. The incorporation of the cyan forming coupler in an amount of 5 to 30 mol% per mole of red-sensitive silver halide can be carried out according to the usual method.

Usable as magenta couplers in the present invention are those illustrated below, but it should naturally be construed that the usable couplers are not limited only thereto.



M-1



M-2



M-3



M-4



M-5



M-6



M-7



M-8

-continued



M-9



M-10



M-11



M-12



M-13



M-14



M-15



M-16

-continued



M-17



M-18



M-19



M-20



M-21



M-22



M-23

-continued



-continued



M-29



M-30



M-31



M-32



M-33

-continued



M-34



M-35



M-36



M-37



M-38



-continued

M-39



M-40



M-41



M-42



M-43

In addition to the magenta couplers as illustrated above, those as usable in the present invention further include such couplers as disclosed, for example, in U.S. Pat. Nos. 3,311,476, 3,419,391 and 3,888,680, West German Patent (OLS) Nos. 2,357,102 and 2,357,122, and Japanese Laid-Open-to-Public Publications Nos. 129538/1974, 23279/1975, 23280/1975, 21687/1975, 127728/1975 and 134470/1975, said couplers may be

60 prepared according to procedures disclosed in these publications, respectively.

The magenta forming couplers used in the present invention may be incorporated into silver halide emulsions, either single or in mixture of two or more, or in admixture with so-called colored couplers, of which the active points have been arylazo-substituted, as disclosed in U.S. Pat. No. 3,005,712. The incorporation of the magenta coupler in an amount of 1 to 25 mol% per mole

of green-sensitive silver halide can be carried out in the usual way.

Usable as oil-soluble photographic additives other than the couplers in the present invention are those as will be mentioned hereinafter.

Usable in the present invention as **DIR** compounds (compounds which produce colorless products on coupling with oxidized color developing agents) are those disclosed, for example, in U.S. Pat. Nos. 3,632,345 and 3,928,041, Japanese Laid-Open-to-Public Publications Nos. 77635/1974, 104630/1974, 36125/1975, 15273/1975, 6724/1976, 23344/1977 and 147716/1975, and Japanese Patent Application No. 2551/1979.

Color stain inhibitors used in the present invention are compounds which are employed for the purpose of inhibiting fog or stain resulting often from unnecessary reaction between oxidized color developing agents resulting from air oxidation and couplers, and these compounds are disclosed, for example, in U.S. Pat. Nos. 2,336,321, 2,360,290, 2,403,721, 2,701,197, 2,728,659 and 3,700,453, British Patent No. 891,158, and Japanese Patent Application No. 2551/1979.

As photofading inhibitors for color dyes used in the present invention, there are those as disclosed, for example, in U.S. Pat. Nos. 3,432,300 and 3,573,050, Japanese Patent Publications Nos. 20977/1974, 31256/1973 and 31625/1973, Japanese Laid-Open-to-Public Publications Nos. 17729/1978 and 48538/1979.

Ultraviolet absorbers used in the present invention include benzotriazoles or benzophenone type compounds as disclosed, for example, in U.S. Pat. Nos. 3,004,896, 3,253,921 and 3,705,805, Japanese Laid-Open-to-Public Publications Nos. 41572/1973 and 25337/1975.

The technique as achieved according to the present invention is applicable to light-sensitive color negative materials, color reversal photosensitive materials, color direct positive photosensitive materials, color paper photosensitive materials, photosensitive materials for instant photography according to DTR process, color X-ray photosensitive materials and black-and-white photosensitive materials. Furthermore, in the case where developers, antioxidants or filter dyes are used, the technology according to the present invention is also applicable to unconventional photosensitive materials. 35 40 45 50

Color photosensitive materials to be prepared according to the present invention may be used as silver halide saving type photosensitive materials as disclosed in West German Patent (OLS) No. 2,357,964 or the like. 50 In processing such photosensitive materials in which the silver halide used has been saved, applicable is a development treatment process as disclosed, for example, in U.S. Pat. Nos. 2,623,822 and 2,814,565, where after halogenation bleaching the developed silver 55 formed by color development, color development is again carried out to increase the dyes formed thereby in amount, a development treatment process using peroxides or utilizing color amplification by the use of cobalt complex salts, or the like development treatment processes. 60

### EXAMPLE 1

A solution was obtained by dissolving 5 g of a yellow coupler of the following formula in a mixture of 5 g of

the present high boiling solvent (35) and 10 g of ethyl acetate while heating the mixture at 70° C. Yellow coupler used:



The solution thus obtained was then incorporated into 60 ml of a 5% gelatin solution containing 0.3 g of sodium dodecylbenzenesulfonate, followed by emulsification dispersing by means of a colloid mill, whereupon a homogeneous and finely emulsified dispersion of the coupler in the solvent was obtained.

Subsequently, the emulsified dispersion thus obtained was incorporated in its entirety into 200 g of a blue-sensitive silver chlorobromide emulsion, followed by addition thereto of a stabilizer and a hardener, and then coated on a baryta paper resin coated with polyethylene to obtain sample 1.

Samples 2 and 3 were obtained by repeating the same procedure as above, except that in place of the present high boiling solvent (35), there were used the present high boiling solvents (34) and (1), respectively. Sample 4 was obtained by repeating the same procedure as above but using the same amount of tricresyl phosphate in place of the present high boiling solvent (35).

Samples 1 through 4 were exposed to light through an optical wedge of the staircase type for sensitometry and then subjected to development treatment in the following manner.

| Color development treatment (31° C.) |                |
|--------------------------------------|----------------|
|                                      | Treatment time |
| Color development                    | 3 minutes      |
| Bleach-fixing                        | 1 minute       |
| Water-washing                        | 2 minutes      |
| Stabilization                        | 1 minute       |
| Water-washing                        | 10 minutes     |
| Drying (below 95° C.)                |                |

Processing solutions used in the steps of the above treatment had their respective compositions as mentioned below.

|                                                                         |         |
|-------------------------------------------------------------------------|---------|
| Composition of color developer solution:                                |         |
| N-Ethyl-N- $\beta$ -methanesulfonamidoethyl-                            |         |
| 3-methyl-4-aminoaniline sulfate                                         | 4.0 g   |
| Hydroxylamine                                                           | 2.0 g   |
| Potassium carbonate                                                     | 25.0 g  |
| Sodium chloride                                                         | 0.1 g   |
| Sodium bromide                                                          | 0.2 g   |
| Anhydrous sodium sulfite                                                | 2.0 g   |
| Benzyl alcohol                                                          | 10.0 ml |
| Polyethylene glycol (average<br>polymerization degree: 400)             | 3.0 ml  |
| Water to make 1 liter and adjusted to pH 10.0 with<br>sodium hydroxide. |         |

|                                        |         |
|----------------------------------------|---------|
| Composition of bleach-fixing solution: |         |
| Iron sodium salt of ethylenediamine-   |         |
| tetraacetic acid                       | 60.0 g  |
| Ammonium thiosulfate                   | 100.0 g |
| Sodium bisulfite                       | 10.0 g  |
| Sodium metabisulfite                   | 3.0 g   |

-continued

Water to make 1 liter and adjusted to pH 6.6 with ammonia water.

Composition of stabilization solution:

|                                 |        |
|---------------------------------|--------|
| Succinic acid                   | g      |
| Formalin (37% aqueous solution) | ml     |
| Water                           | 800 ml |

Adjust the pH to 3.9 with sodium acetate and then bring the solution up to 1 liter with the addition of water.

On the other hand, the exposed samples 1 through 4 were subjected to development treatment in the same manner and same conditions as above, except that in the step of color development, the color developer solution from which the benzyl alcohol had been excluded was used.

Yellow images respectively obtained on the thus processed samples were measured in speed, fog and maximum density (Dmax) by means of a densitometer (Model KD-7R, manufactured by Konishiroku Photo Industry Co., Ltd.) to obtain the results as shown in table 1, wherein the speed was represented by a relative value as measured by assuming as 100 the speed of sample 4 containing the comparative high boiling solvent (TCP) and processed with the color developer solution containing 10.0 ml of benzyl alcohol.

TABLE 1

| Sam-<br>ple<br>No. | High<br>boiling<br>solvent | Benzyl alcohol<br>10 ml/l |      |      | Benzyl alcohol<br>0/1 |      |      |
|--------------------|----------------------------|---------------------------|------|------|-----------------------|------|------|
|                    |                            | Speed                     | Fog  | Dmax | Speed                 | Fog  | Dmax |
| 1                  | Exemplified compound 35    | 125                       | 0.08 | 2.96 | 83                    | 0.06 | 2.56 |
| 2                  | Exemplified compound 34    | 128                       | 0.07 | 2.90 | 85                    | 0.06 | 2.48 |
| 3                  | Exemplified compound 1     | 115                       | 0.07 | 2.80 | 75                    | 0.06 | 2.30 |
| 4                  | Comparative compound (TCP) | 100                       | 0.08 | 2.70 | 45                    | 0.05 | 1.75 |

From table 1, it is understood that in the benzyl alcohol-containing color development treatment, samples 1 through 3 comprising the present high boiling solvents were found to be superior in color developability to sample 4 comprising the comparative high boiling solvent (TCP). Even in the color development treatment where no benzyl alcohol was used, moreover, the present samples 1 through 3 apparently increased in color developability as compared with the comparative sample 4, and thus it is understood that light-sensitive color photographic materials comprising the present high boiling solvents are less dependent in their developability on the use of benzyl alcohol in color developer solutions.

Furthermore, from the fact that the samples 1 and 2 greatly increased in color developability by comparison with the sample 3, it is understood that even in the present high boiling solvents, those having substituted alkyl groups are superior to those having unsubstituted alkyl groups so far as color developability is concerned.

Separately, the samples 1 through 4 processed with the benzyl alcohol-containing developer solution were subjected for 8 days to irradiation by means of a xenon

fade-o-meter to investigate light fastness of color images formed on the samples, respectively. The results obtained were as shown in table 2, wherein the evaluation of light fastness was represented by percent residual dye as measured at the initial density 1.0 and by percent residual dye as measured after the light fastness test at the Dmax area of each color image.

TABLE 2

| Sample | High boiling solvent       | Initial density         |                                     |
|--------|----------------------------|-------------------------|-------------------------------------|
|        |                            | (1.0)<br>% residual dye | (D <sub>m</sub> )<br>% residual dye |
| 1      | Exemplified compound 35    | 88                      | 90                                  |
| 2      | Exemplified compound 34    | 90                      | 87                                  |
| 3      | Exemplified compound 1     | 85                      | 85                                  |
| 4      | Comparative compound (TCP) | 75                      | 75                                  |

As is clear from table 2, it is understood that the samples 1 through 3 comprising the present high boiling solvents are greatly improved in light fastness in comparison with the sample 4 comprising the comparative high boiling solvent (TCP).

## EXAMPLE 2

Using the present exemplified compound (M-2) as a magenta couple, emulsified coupler dispersions were individually prepared as prescribed below.

|                                |       |
|--------------------------------|-------|
| Magenta coupler                | 10 g  |
| Photofading inhibitor*         | 3 g   |
| High boiling organic solvent   | 10 g  |
| Ethyl acetate                  | 20 g  |
| Sodium dodecylbenzenesulfonate | 0.3 g |
| 5% gelatin solution            | 60 ml |

\*Photofading inhibitor 1,4-di-octyloxy-2,5-dipentylbenzene

That is, each emulsified dispersion was prepared by dissolving the magenta coupler and photofading inhibitor in a mixture comprising each of the under-mentioned high boiling organic solvents and ethyl acetate while heating the mixture at 70° C. and emulsifying and dispersing the resulting solution in a 5% gelatin solution containing sodium dodecylbenzenesulfonate by means of a colloid mill. The whole of the emulsified dispersion was incorporated into 200 g of a green-sensitive silver chlorobromide emulsion, followed by addition thereto of a stabilizer and a hardener, and the emulsion was coated on a baryta paper resin-coated with polyethylene and then dried.

[High boiling organic solvent used]

Exemplified compounds (39) (32) (9)

Comparative compounds (A): Dibutyl phthalate (DBP)  
Comparative compounds (B): Triamyl phosphate (TAP)

Samples 5 through 9 obtained in the above manner were exposed to light and then subjected to development treatment in the same way as in Example 1 to obtain magenta images on the samples, respectively. The samples thus processed were subjected to irradiation for 8 days by means of a xenon fade-o-meter to investigate light fastness of the color image and yellow stain of the uncolored portion. Further, the samples thus color developed were individually measured in spectrophotometry by means of a spectrophotometer

(manufactured by Hitachi, Ltd.), the measured value of spectroreflectance was converted into to measure spectral absorption property, whereby values of adsorption maximum and red light adsorption were determined.

TABLE 3

| Sam-<br>ple | High boiling<br>solvent    | Light<br>fastness           |              | Ab-<br>sorp-<br>tion<br>max-<br>imum | Absorption<br>( $\Delta\lambda/\Delta\lambda_{max}$ )<br>$\lambda = 600nm$ | $\lambda = 620nm$ |
|-------------|----------------------------|-----------------------------|--------------|--------------------------------------|----------------------------------------------------------------------------|-------------------|
|             |                            | Initial<br>density<br>(1.0) | Stain<br>(%) |                                      |                                                                            |                   |
| 5           | Exemplified compound 39    | 85                          | 0.19         | 550                                  | 0.39                                                                       | 0.22              |
| 6           | Exemplified compound 32    | 83                          | 0.20         | 549                                  | 0.38                                                                       | 0.21              |
| 7           | Exemplified compound 9     | 86                          | 0.24         | 550                                  | 0.39                                                                       | 0.22              |
| 8           | Comparative compound (DBP) | 72                          | 0.28         | 555                                  | 0.45                                                                       | 0.25              |
| 9           | Comparative compound (TAP) | 83                          | 0.23         | 551                                  | 0.40                                                                       | 0.22              |

From table 3, it is understood that as compared with sample 8 comprising the comparative compound (DBP), samples 5 through 7 comprising the present high boiling solvents and sample 9 comprising the comparative compound (TAP) were distinctly improved in light fastness as well as in stain of the uncolored portion.

It is further understood that as is appreciably different from the case of the comparative sample 9, the dominant wavelength in each of the samples 5-7 and in the comparative sample 8 shifted to a shorter wavelength region, thereby improving distinctly sub-absorption at a wavelength above 600 nm.

## EXAMPLE 3

Using a cyan coupler represented by following formula, emulsified coupler dispersions were individually prepared as prescribed below. Cyan coupler used:

|                                |
|--------------------------------|
|                                |
| Cyan coupler                   |
| High boiling organic solvent   |
| Ethyl acetate                  |
| Sodium dodecylbenzenesulfonate |
| 5% Gelatin solution            |

That is, each emulsified dispersion was obtained by dissolving the cyan coupler in a mixture comprising each of the under-mentioned high boiling organic solvents and ethyl acetate while heating the mixture at 70° C. and emulsifying and dispersing the resulting solution in a 5% gelatin solution containing sodium dodecylbenzenesulfonate by means of a colloid mill. The whole of the emulsified dispersion was incorporated into 200 g of a red-sensitive silver chlorobromide emulsion, followed by addition thereto a stabilizer and a hardener, and the emulsion was coated on a baryta paper resin-coated with polyethylene and then dried.

[High boiling organic solvent used]

Exemplified compounds (6) (28)

Comparative compound: Dibutyl phthalate (DBP)

Samples 10 through 12 thus prepared were exposed and developed in the same procedure as in Example 1 to obtain colored samples. The colored samples were individually subjected to preservation test for color image after having been stored for 2 weeks at 60° C. and 80% RH and for 2 weeks at 77° C. and dry, respectively, to obtain the results as shown in table 4, wherein the preservative properties of the color image was expressed in terms of percent residual dye as measured after storage at the initial density = 1.0, and the green discoloration degree was represented by the difference (B/R after storage-B/R before storage).

TABLE 4

| Sample<br>No. | High boiling<br>solvent    | 60° C. 80% RH<br>(D = 1.0) |      | 77° C. Dry<br>(D = 1.0) |      |
|---------------|----------------------------|----------------------------|------|-------------------------|------|
|               |                            | Residual<br>dye %          | B/R  | Residual<br>dye %       | B/R  |
| 10            | Exemplified compound 6     | 83                         | 0.09 | 81                      | 0.10 |
| 11            | Exemplified compound 28    | 85                         | 0.08 | 83                      | 0.11 |
| 12            | Comparative compound (DBP) | 63                         | 0.15 | 60                      | 0.20 |

As is clear from table 4, it is understood that in comparison with the sample 12 comprising the comparative compound (DBP), the samples 10 and 11 comprising the present high boiling organic solvents, respectively, distinctly improved preservative properties of the color image thereof.

## EXAMPLE 4

Using the present exemplified compound (M-20) as a magenta coupler, emulsified coupler dispersions were individually prepared as prescribed below.

|                                |       |
|--------------------------------|-------|
| Magenta coupler                | 10 g  |
| High boiling organic solvent   | 10 g  |
| Ethyl acetate                  | 20 g  |
| Sodium dodecylbenzenesulfonate | 0.3 g |
| 5% Gelatin solution            | 60 ml |

That is, each emulsified coupler dispersion was obtained by dissolving the magenta coupler in a mixture comprising each of the under-mentioned high boiling organic solvent and ethyl acetate while heating the mixture at 70° C. and emulsifying and dispersing the resulting solution in a 5% gelatin solution containing sodium dodecylbenzenesulfonate by means of a colloid mill. The whole of the emulsified dispersion was incorporated into 200 g of a green-sensitive silver iodobromide emulsion, followed by addition thereto of a stabilizer and a hardener, and the emulsion was coated on a cellulose triacetate film base and then dried.

[High boiling organic solvent used]

Exemplified compounds (22) (32) (33)

Comparative compound (A): Tricresyl phosphate (TCP)

Comparative compound (B): Triacyl phosphate (TAP)

Samples 13 through 17 obtained in the above manner were subjected to exposure to light in the usual way and then color developed according to the following processing steps.

| Processing step (38° C.) |                 | 5  | Dmax as measured after ordinary development treatment          |       | × 100. |
|--------------------------|-----------------|----|----------------------------------------------------------------|-------|--------|
|                          | Processing time |    | Dmax as measured after treatment with ferricyanide bleach bath |       |        |
| Color development        | 3' 15"          |    |                                                                |       |        |
| Bleaching                | 6' 30"          |    |                                                                |       |        |
| Water-washing            | 3' 15"          |    |                                                                |       |        |
| Fixing                   | 6' 30"          |    |                                                                |       |        |
| Stabilization            | 1' 30"          |    |                                                                |       |        |
|                          |                 | 10 | Prescription of ferricyanide bleach bath                       |       |        |
|                          |                 |    | K <sub>3</sub> Fe(CN) <sub>6</sub>                             | 95 g  |        |
|                          |                 |    | K <sub>4</sub> Fe(CN) <sub>6</sub>                             | 6.5 g |        |
|                          |                 |    | Nitrotriacetate                                                | 18 g  |        |
|                          |                 |    | KBr                                                            | 25/1  |        |

Processing solutions used in the above-mentioned steps had their respective compositions as shown below:

|                                                                       |         |  |  |  |  |
|-----------------------------------------------------------------------|---------|--|--|--|--|
| [Composition of color developer solution]                             |         |  |  |  |  |
| 4-Amino-3-methyl-N—ethyl-N—(β-hydroxyethyl)-aniline sulfate           | 4.75 g  |  |  |  |  |
| Anhydrous sodium sulfite                                              | 4.25 g  |  |  |  |  |
| Hydroxylamine ½ sulfate                                               | 2.0 g   |  |  |  |  |
| Anhydrous potassium carbonate                                         | 37.5 g  |  |  |  |  |
| Potassium bromide                                                     | 1.3 g   |  |  |  |  |
| Nitrotriacetic acid trisodium salt (monohydrate)                      | 2.5 g   |  |  |  |  |
| Sodium hydroxide                                                      | 1.0 g   |  |  |  |  |
| Water to make 1 liter and adjust to pH 10.0 with potassium hydroxide. |         |  |  |  |  |
| [Composition of bleaching solution]                                   |         |  |  |  |  |
| Iron ammonium salt of ethylene-diaminetetraacetic acid                | 100.0 g |  |  |  |  |
| Diammonium salt of ethylene-diaminetetraacetic acid                   | 10.0 g  |  |  |  |  |
| Ammonium bromide                                                      | 150.0 g |  |  |  |  |
| Glacial acetic acid                                                   | 10.0 ml |  |  |  |  |
| Water to make 1 liter and adjust pH to 6.0 with ammonia water.        |         |  |  |  |  |
| [Composition of fixing solution]                                      |         |  |  |  |  |
| Ammonium thiosulfate (50% aqueous solution)                           | 152 ml  |  |  |  |  |
| Anhydrous sodium sulfite                                              | 12.4 g  |  |  |  |  |
| Water to make 1 liter and adjust pH to 6.5 with acetic acid.          |         |  |  |  |  |
| [Composition of stabilizing solution]                                 |         |  |  |  |  |
| Formalin (37% aqueous solution)                                       | 5.0 ml  |  |  |  |  |
| Konidax (produced by Konishiroku Photo Industry Co., Ltd.)            | 7.5 ml  |  |  |  |  |
| Water to make 1 liter.                                                |         |  |  |  |  |

Magenta images obtained respectively on the samples thus developed under the above-mentioned conditions were subjected to sensitometry by means of a densitometer (Model KD-7R manufactured by Konishiroku Photo Industry Co., Ltd.) to obtain the results with respect to speed, fog and maximum density (Dmax) as shown in Table 5, wherein the speed was represented by a relative value as measured by assuming as 100 the speed of the sample 16 comprising the comparative compound (A).

Furthermore, after having been subjected to sensitometry, the developed samples were again subjected to sensitometry in order to investigate dye forming rate of the magenta coupler during the above-mentioned color development treatment, after immersing said developed samples at 20° C. for 5 minutes in a ferricyanide containing bleach bath as prescribed below to obtain the result as shown in table 5, wherein the dye forming rate was represented by a value obtained from the calculation of

| 15 | Sample No. | High boiling solvent       | Speed | Fog  | Dmax | Dye forming rate |
|----|------------|----------------------------|-------|------|------|------------------|
|    | 13         | Exemplified compound 22    | 130   | 0.14 | 2.10 | 97               |
|    | 14         | Exemplified compound 32    | 127   | 0.12 | 2.16 | 98               |
|    | 15         | Exemplified compound 33    | 123   | 0.12 | 2.08 | 97               |
|    | 16         | Comparative compound (TCP) | 100   | 0.11 | 1.60 | 72               |
|    | 17         | Comparative compound (TAP) | 115   | 0.12 | 1.80 | 85               |

As is clear from table 5, it is understood that in comparison with the samples 16 and 17 comprising the comparative compounds TCP and TAP, respectively, the samples 13 through 15 comprising the present high boiling organic solvents are excellent in treatment stability as evidenced by their being high in both speed and Dmax as well as in dye forming rate.

On the other hand, the samples 13 through 17 as prepared, which had remained unexposed, were stored for 3 months under natural conditions (25° C. 60% RH) and thereafter exposed and developed in the same manner as above to obtain their respective colored samples. The colored samples thus obtained were investigated with respect to their preservative properties of raw film 40 in comparison with the samples 13 through 17 as prepared, which had been exposed and developed immediately after preparation thereof. The results obtained were as shown in table 6.

| 45 | Sam- ple No. | Speed                         |                            | Dmax                          |                            |
|----|--------------|-------------------------------|----------------------------|-------------------------------|----------------------------|
|    |              | Immediately after preparation | After storage for 3 months | Immediately after preparation | After storage for 3 months |
| 50 | 13           | 130                           | 125                        | 2.10                          | 2.06                       |
|    | 14           | 127                           | 120                        | 2.16                          | 2.00                       |
|    | 15           | 123                           | 126                        | 2.08                          | 2.20                       |
|    | 16           | 100                           | 98                         | 1.60                          | 1.63                       |
|    | 17           | 115                           | 50                         | 1.80                          | 1.35                       |

As is clear from table 6, it is understood that in comparison with the sample 17 comprising the comparative high boiling solvent (B), the samples 13 and 14 comprising the present high boiling solvents, respectively, were markedly improved in preservative properties of raw film.

#### EXAMPLE 5

Emulsified coupler dispersions were prepared in the same prescription and procedure as in Example 4 using 65 as magenta couplers the present exemplified magenta couplers M-22, M-23, M-27, M-30 and M-41, and the present high boiling solvent compounds (11), (37), (42), (44) and a comparative high boiling solvent (TCP), and

the resulting dispersions were individually coated on a support to obtain samples 18 through 22. The samples thus obtained were exposed and developed in the same manner as in Example 4 to investigate Dmax and dye forming rate (dependability on processing solution) of each coupler. The results obtained were as shown in table 7.

TABLE 7

| Sample No. | Present coupler | High boiling solvent       | Dmax | Dye forming rate (%) |
|------------|-----------------|----------------------------|------|----------------------|
| 18         | M-22            | Exemplified compound 11    | 2.23 | 96                   |
| 19         | M-23            | Exemplified compound 37    | 2.15 | 97                   |
| 20         | M-27            | Exemplified compound 42    | 2.30 | 100                  |
| 21         | M-30            | Exemplified compound 44    | 2.28 | 97                   |
| 22         | M-40            | Comparative compound (TCP) | 1.65 | 73                   |

From table 7, it is understood that the samples 18 through 21 each comprising the present high boiling solvent having dissolved therein the present bis type magenta coupler are all found excellent in color development as well as in dye forming rate of the coupler.

## EXAMPLE 6

Using the present exemplified compound (M-26) as a magenta coupler, emulsified dispersions were prepared according to the following prescription.

|                                |       |
|--------------------------------|-------|
| Magenta coupler                | 10 g  |
| DIR compound*                  | 1 g   |
| High boiling solvent           | 10 g  |
| Ethyl acetate                  | 20 g  |
| Sodium dodecylbenzenesulfonate | 0.3 g |
| 5% Gelatin solution            | 60 ml |

\*DIR compound 2-(1-phenyl-5-tetrazolylthio)-4-(2,4-di-t-amylphenoxyacetamido)-1-indanone

That is, each emulsified coupler dispersion of the magenta coupler and the DIR compound was prepared in the same manner as in Example 4, and the resulting dispersion was incorporated into 200 g of a green-sensitive silver bromide emulsion, followed by addition thereto of a stabilizer and a hardener. The emulsion was coated on a cellulose acetate film base and then dried.

[High boiling organic solvent used]

Exemplified compound (11)

Comparative compound: Tricresyl phosphate

Samples 23 and 24 obtained in the above manner were exposed and developed in the same manner as in Example 4 to investigate photographic properties thereof, whereupon the sample comprising the present high boiling solvent showed excellent photographic properties.

What we claim is:

1. A silver halide photographic material having a support and a hydrophilic colloidal layer coated thereon, said hydrophilic colloidal layer containing a solution of (a) a 5-pyrazolone type magenta coupler;

and (b) a high-boiling organic solvent having the general formula [I]:



wherein R<sub>1</sub>, R<sub>2</sub> and R<sub>3</sub> each represent an aliphatic or aromatic group and a carbon atom of R<sub>3</sub> is bonded directly to the phosphorus atom.

2. A silver halide photographic material having a support and a hydrophilic colloidal layer coated thereon, said hydrophilic colloidal layer containing a solution of (a) an aldehyde-bis 5-pyrazolone type magenta coupler (b) a high-boiling organic solvent having the general formula [I]:



wherein R<sub>1</sub>, R<sub>2</sub> and R<sub>3</sub> each represent an aliphatic or aromatic group and a carbon atom of R<sub>3</sub> is bonded directly to the phosphorus atom.

3. The silver halide photographic material of claim 1 or 2 wherein said solvent is dispersed in the hydrophilic colloidal layer.

4. The silver halide photographic material of claim 1 or 2 wherein R<sub>1</sub>, R<sub>2</sub> and R<sub>3</sub>, which may be the same or different, each represent an alkyl or aryl group, and the sum of carbon atoms of R<sub>1</sub>, R<sub>2</sub>, and R<sub>3</sub> is in the range from 6 to 50.

5. The silver halide photographic material of claim 3, wherein the substituent R<sub>3</sub> has a carbonyloxy-carbonamido-containing group or an alkoxyalkyl, aryloxyalkyl, alkoxyaryl, arylalkyl or acylalkyl group.

6. A process for incorporating an oil-soluble photographic additive into a hydrophilic colloidal solution for forming a photographic colloidal layer, comprising the steps of:

(a) dissolving the oil-soluble photographic additive in a high-boiling organic solvent having the general formula [I]:



wherein R<sub>1</sub>, R<sub>2</sub> and R<sub>3</sub> each represents an aliphatic or aromatic group, and a carbon atom of R<sub>3</sub> is bonded directly to the phosphorus atom, to obtain a first solution; and

(b) thereafter incorporating said first solution into said hydrophilic colloidal solution.

7. The process of claim 6 wherein said first solution is dispersed in said hydrophilic colloidal solution.

8. The process of claim 6 wherein said oil-soluble additive is a coupler, a DIR compound, a UV-absorbing agent, a photofading inhibitor or an anti-staining agent.

\* \* \* \* \*